

## UNITED STATES PATENT OFFICE

1,957,420

CINEMATO-PHONOGRAPHIC  
PHOTOGRAPHY

Pierre Butez, Vaucresson, and Pierre Contant,  
Courbevoie, France, assignors to Societe Inde-  
pendante de Telegraphie Sans Fil, Malakoff,  
France

No Drawing. Application March 27, 1930, Serial  
No. 439,527. In France March 27, 1929

3 Claims. (Cl. 95—88)

The present invention relates to cinematophono-  
graphic photography.

Cinematophono-graphic methods are known in  
which the entire film surface is covered with a  
5 photographic image adapted to be projected and  
an acoustic image or record, the former being  
composed of a substance opaque to visible and  
transparent to invisible radiations and the latter  
of a substance opaque to invisible and transparent  
10 to visible radiations.

The object of the invention is to provide a  
method for treating metallic photographic  
(acoustic) images so as to substitute a cupric salt,  
such as cupric chloride or sulphate, such salt be-  
15 ing transparent to visible and opaque to infra-red  
radiations for the usual silver image.

The method may be carried out as follows:

The silver of the acoustic image or record is  
first transformed into silver ferrocyanide by  
20 means of an ammoniacal solution of potassium  
ferricyanide. After washing to eliminate the  
excess ferricyanide and the potassium formed,  
the film is submerged in a bath of cupric chlo-  
ride. The silver ferrocyanide is gradually trans-  
25 formed into the corresponding cupric salt with  
formation of silver chloride which may be re-  
moved by means of a solution of ammonium  
sulphocyanide. The cupric ferrocyanide formed  
on the film is then treated with caustic alkali  
30 solution to form cupric hydroxide which is fin-  
ally converted into the corresponding chloride or  
sulphate by means of hydrochloric or sulphuric  
acid.

The final film may include silver, copper, plat-  
35 inum, asphalt, or any other substance opaque to  
visible and transparent to invisible radiations.

It is to be understood that the foregoing meth-  
ods are applied to film in which the ordinary  
40 supporting surface, the silver acoustic image be-  
ing superposed on the ordinary photographic  
image.

What we claim is:—

1. The method of treating a film having a photo-  
graphic record of known type and an acoustic  
silver record mutually superposed which in a  
combined group of steps consists in treating the 60  
silver acoustic record with an ammoniacal solu-  
tion of potassium ferricyanide, washing, then  
treating the film first with a cupric chloride solu-  
tion and subsequently with an ammonium sul-  
phocyanide solution, and finally immersing the 65  
film in an alkaline solution in order to produce  
a cupric hydroxide.

2. The method of treating a film having a photo-  
graphic record of known type and an acoustic  
silver record mutually superposed which in a 70  
combined group of steps consists in treating the  
silver acoustic record with an ammoniacal solu-  
tion of potassium ferricyanide, washing, then  
treating the film successively with a cupric chlo-  
ride solution and an ammonium sulphocyanide 75  
solution, immersing the film in an alkaline solu-  
tion to produce a cupric hydroxide, and finally  
treating the film with a solution of sulphuric acid  
in order to convert the cupric hydroxide into  
cupric sulphate.

3. The method of treating a film having a photo-  
graphic record of known type and an acoustic  
silver record mutually superposed which in a  
combined group of steps consists in treating the 85  
silver acoustic record with an ammoniacal solu-  
tion of potassium ferricyanide, washing, then  
treating the film successively with a cupric chlo-  
ride solution and an ammonium sulphocyanide  
solution, immersing the film in an alkaline solu- 90  
tion to produce a cupric hydroxide in said film,  
and finally treating the film with a solution of  
hydrochloric acid in order to convert the cupric  
hydroxide therein into cupric chloride.

PIERRE BUTEZ.  
PIERRE CONTANT.